

Patented Sept. 28, 1926.

1,601,244

# UNITED STATES PATENT OFFICE.

RICHARD FALCK, OF MUNDEN IN HANOVER, GERMANY.

## PROCESS FOR THE PRODUCTION OF SOLID ALCOHOL STRUCTURE SOAPS.

No Drawing. Application filed December 5, 1924, Serial No. 754,162, and in Germany November 12, 1923.

The solid alcohol soaps on the market are either in the shape of a handy tablet of solid soap, like toilet soap, or of paste which for use is filled in tubes. These soaps serve for 5 washing and disinfecting purposes and are well adapted, especially when in pasty state, to form carriers for medicinal substances. The solid soap cakes make a homogeneous 10 jelly-like impression and resemble still the ordinary water containing soap. They still possess considerable solidity and a comparatively high melting point above the warmth of the body. To the solidity corresponds however a certain brittleness; the 15 soaps break into round lumps when a knife is stuck into them or even under a strong pressure. The alcohol is not yet sufficiently bound in the same and it can be easily removed by pressure or suction. The pasty 20 soaps are of limited durability as, probably owing to the pressure exerted at the preparation, a separation of the liquid and solid constituents takes place after a comparatively short time. While for instance directly 25 after the preparation of the paste from the soap and after the filling into tubes an absolutely uniform jet can be pressed out of the tubes. After some weeks it will be seen that, a liquid will flow out of the tube, besides the 30 paste, said paste consisting of alcohol or liquid soap-alcohol.

Experiments have shown that the products made in the apparatus of known type preserve the characteristics mentioned however 35 the proportions of the constituents may be varied. If however soaps which have been desiccated to about 5% water and 96% ethyl alcohol in a proportion in which they are no longer capable to be dissolved in the commonly used apparatus e. g. in open vessels, 40 are heated in closed vessels, for instance in an autoclave, at increased atmospheric pressure and at a temperature above the boiling point of the alcohol, products are obtained 45 which, as regards physical properties and the effect resulting from the same, differ considerably from the production hitherto obtained.

The products from the mixtures mentioned of desiccated soap and alcohol of high percentage which must be heated in closed vessels in order that they are able to form a solution, can no longer be moulded, as the commonly used soaps do, by being poured 50 into open molds in the free air as an alcohol soap of 25% Na-laurate, 5% Na-stearate, 5%

Na-palmitate, 2.5% Na-oleate and 62.5% alcohol will for instance melt in the usual melting point apparatus in a capillary tube closed by melting, without fail at 100° to 60 110° C., that is considerable above the boiling point of alcohol. In solidified condition the products mentioned solidify already at a comparatively high temperature. They form then an opaque streaky-thready mass, similar 65 to fungus flesh, which is not in the least like the hitherto known structureless soap jellies. Observed under the microscope the new substance looks generally as consisting of an aggregate of fine needle-like or granulous elements which are intertwined in a felt-like manner.

In the new product the alcohol is incorporated in the soap so well that the separation of the same from the paste produced 75 under pressure does no longer interfere with the usefulness and the melting point is higher and therefore more favorable than in the soaps on the market. The solid tablet does no longer decompose into round lumps even under strong pressure and it can be worked 80 with the knife like ordinary soap. If the soap chips are dried in the air they preserve the same streaky character while the residues of soap from the alcohol soap prepared according to the hitherto used methods are 85 after the evaporation of the alcohol which they contain like a more or less aged silicic acid jelly.

The process can be carried out as follows:—

45 parts of chipped soaps, desiccated to about 5%, are heated together with 55 parts of alcohol of 96 volume percent in an autoclave at a temperature of 120° C. and 95 at a pressure of 6 atms. for 1½ hours. After cooling a very hard alcohol-structure-soap is obtained the melting point of which is about 90° C., said soap giving up under the suction pump only very little alcohol even 100 when being compressed and it is capable of being treated with a knife without disintegrating. 10 gr. of a paste composed of 26.3% desiccated soap and 73.7% alcohol have, for instance, been exposed at a reduced 105 pressure of 50 mm. in the suction bottle for 10 minutes to the action of the suction pump. 1.5 c. cm. cube of alcohol were sucked off or about 19% of the alcohol contained in the soap.

110 By mixing the micro produced structure-alcohol-soap with the hitherto used struc-

tureless jelly soap preparations in pasty form can be obtained which are preferably designed for medical purposes. These soaps soften when rubbed into the skin and penetrate also into deeper layers of the skin as the alcohol contained in the soaps, besides its disinfecting property dissolves the fatty, resinous and slimy substances which choke up the pores of the skin and makes these pores free to admit the alcohol soap. This is true of all kinds of mixtures of alcohol soaps however much the proportion of the sebacic salts of the soap may vary in the fundamental soaps, and also when medicinal substances are added to the alcohol soaps.

I claim:—

A process for the production of solid alcohol soap containing a high percentage of alcohol by heating soap almost completely freed from water in alcohol of great <sup>20</sup> strength, comprising the steps that a mixture of about 45 parts by weight of soap and about 55 parts by weight of alcohol is heated in a closed vessel at a temperature of 120° C. and under a pressure of 6 atms., and <sup>25</sup> in continuing the heating under pressure for one hour and one-half so that the product obtained contains the total quantity of alcohol of the mixture.

In testimony whereof I affix my signature.

DR. RICHARD FALCK.